

# UNITED STATES PATENT OFFICE.

SHIPLEY NEAVE BRAYSHAW, OF HULME, MANCHESTER, ENGLAND,  
ASSIGNOR TO GEORGE NASH, OF NEW YORK, N. Y.

## PROCESS OF HARDENING STEEL.

No. 838,375.

Specification of Letters Patent.

Patented Dec. 11, 1906.

Application filed June 8, 1906. Serial No. 320,876.

*To all whom it may concern:*

Be it known that I, SHIPLEY NEAVE BRAYSHAW, a subject of the King of England, and a resident of Hulme, Manchester, county of Lancaster, England, have invented certain new and useful Improvements in the Process of Hardening Steel, of which the following is a specification.

In the ordinary method of hardening ordinary or carbon steel it has been heated in a furnace or otherwise to a certain temperature, known as the "hardening-point," which varies according to the composition of the steel, and then quenched in a cold or cool bath of water, oil, or other liquid. I now find that better results are obtained by heating the steel to a temperature considerably above the hardening-point and then reducing it to a point somewhat below the hardening-point and finally quenching in a cold bath, such as water, brine, or oil.

I have discovered that if carbon steel is highly heated a remarkable change occurs at a temperature of about  $140^{\circ}$  centigrade beyond the hardening-point. This change occurs at what I call the "higher-change" point, and the temperature of this is usually about  $880^{\circ}$  centigrade. If the steel bars are heated to the higher-change point and then quenched in water, they are found to be the same length after quenching as they were before the heating began. There are various other effects due to raising carbon steel to the higher-change point. For instance, the appearance of the fracture of the steel is altered very considerably and the value of the steel for many kinds of tools and other articles is enormously increased. I have discovered, further, that after carbon steel has been heated to the higher-change point it may be lowered to a temperature considerably below the ordinary hardening-point, and it will still harden if quenched from this lower temperature. Moreover, it retains many of the properties which it acquired while it was at the higher-change point.

I am well aware that carbon steel has frequently been heated up to or above the ordinary hardening-point and then lowered in temperature below the hardening-point before being quenched and that steel so treated has been hardened; but I find that if steel which has not been heated to the higher-change point is lowered below the ordinary

hardening-point it will soon acquire the condition corresponding to this low temperature, and even a short soaking at this low temperature will bring it into a condition in which it will not harden when quenched. Now after I have raised the carbon steel to the higher-change point I can lower it as much as  $20^{\circ}$  centigrade (and in some cases a good deal more) below the hardening-point and soak it at this low temperature for a prolonged period, (sometimes as long as several hours,) and it will still harden if quenched. I find that when carbon steel is raised to the higher-change point and then lowered to a certain temperature below the hardening-point and then quenched in water it hardens without any risk of cracking, and steel which has been hardened in this way possesses valuable cutting and other properties which cannot be given to it by any other means.

The term "carbon steel" as I use it in this specification is meant to include carbon steels which contain a small percentage of alloy, and it is used as an antithesis to the term "high-speed steel."

In carrying out the invention I heat the articles in a bath at a very high temperature, considerably above the hardening-point, so as to reach or pass a certain higher-change point. Thus for a steel of which the hardening-point is, say,  $740^{\circ}$  centigrade I should heat up to from  $860^{\circ}$  to  $900^{\circ}$  centigrade. The article is soaked in this bath from a few seconds up to many minutes, according to the size and bulk, until it is uniformly heated up to the full temperature. The article is then removed and immediately immersed in a second bath (care being taken not to allow it to cool) at a temperature somewhat below the hardening-point—say about  $705^{\circ}$  to  $730^{\circ}$  centigrade. The article may be soaked in this second bath for a considerable length of time—about the same length of time as in the first bath, or until uniformly reduced in temperature to the heat of the second bath. The relative lengths of times, however, for soaking in the two baths are partly dependent upon the temperatures thereof and may be varied considerably. After soaking in the second bath the article is removed and quenched out in a cold bath of water, brine, oil, or other liquid, (say about  $20^{\circ}$  centigrade.) The article may be cold when placed in the

first high-temperature bath, or it may be previously heated in another bath or otherwise; but any preliminary heating must not reach a temperature higher than the temperature of the first bath. Instead of immersing the articles in the first bath for the whole time of heating it sometimes happens that I alternately lower them into and lift them out of the bath and keep doing this for all or part of the time of heating until they are brought to a temperature uniform with the bath. As a rule the articles are immersed continuously for the whole time in the second bath.

15 The process may be carried out and the bath heated in a furnace such as that described in the specification of my former patent, No. 769,052 of 1903, or the bath may be heated to the desired degree in any other form 20 of furnace. I prefer the bath to be composed of fused salts; but molten lead or alloy may be used. The temperatures of the baths vary according to the composition of the steel under treatment and also to a slight 25 degree according to the size of the articles under treatment. When the article has been correctly heated to the high temperature and then lowered as described, there is no risk of breakages, even though the temperatures of the baths have varied by an 30 amount that was fatal to the work when it was hardened at one heat only. This process of hardening allows a greater range of

variation in the temperature than formerly, and by it I secure an intense hardness of the article so treated, and I find that tools so hardened last much longer and do much more work than any tools previously made of ordinary carbon steel.

What I claim as my invention, and desire to protect by Letters Patent, is—

1. The process of hardening ordinary carbon steel which consists in heating the article in a bath so as to reach a certain higher-change point at a temperature considerably 45 above the hardening-point, then soaking it for a considerable time in a bath somewhat below the hardening-point and subsequently quenching in a cold bath substantially as described.

2. The process of hardening ordinary carbon steel with a hardening-point of about 740° centigrade which consists in heating in a bath to reach a certain higher-change point at a temperature of 860° to 900° centigrade, 55 then soaking for a considerable time in a cooler bath at a temperature of 705° to 730° centigrade and finally quenching in an ordinary cold bath substantially as described.

In witness whereof I have hereunto signed my name in the presence of two subscribing witnesses.

SHIPLEY NEAVE BRAYSHAW.

Witnesses:

J. OWDEN O'BRIEN,  
H. BARNFATHER.